

## UNITED STATES PATENT OFFICE

GELLERT ALLEMAN, OF SWARTHMORE, PENNSYLVANIA, ASSIGNOR TO SUN OIL COMPANY, OF PHILADELPHIA, PENNSYLVANIA, A CORPORATION OF NEW JERSEY

## COLORED GASOLINE

No Drawing.

Application filed July 28, 1928. Serial No. 296,101.

In the sale of gasoline at retail under a trade-mark, or as the advertised product of a particular manufacturer, it is important that the purchaser shall receive the precise product for which he asks. Unless, however, the manufacturer operates his own filling stations, there is nothing to prevent an unscrupulous retailer from substituting a cheaper and inferior gasoline, thereby damaging the reputation of the manufacturer and inflicting upon him serious loss, the extent of which it is difficult to compute.

The prevention of this substitution of inferior gasoline for superior gasoline by imparting to the gasoline a peculiar and distinctive color which it will be difficult or practically impossible for the vendor to impart to any uncolored gasoline is one of the objects of the invention. This problem presents serious difficulties. The color must not be one which will impart any cloudy appearance to the gasoline. The color must not be one that characterizes inferior gasoline, or which is, rightly or wrongly, associated, in the mind of the purchasing public, with inferior gasoline. The color must be fast; that is, must not change on exposure to light or during storage for a shorter or longer time. The gasoline should not be colored with a dye that, if the gasoline is used for dry cleaning, will impart an objectionable color to the garments. The color must also be insoluble in water for reasons hereinafter stated. The gasoline must be carefully refined in order to prevent an otherwise fast color from being ineffective to maintain the color imparted by the gasoline.

The coloring of petroleum products by means of different dyes and coloring matters is well known. Most of these colors or dyes, when mixed with oil, will, when water is subsequently added, leave the oil, in whole or in part, and go into the water. Some of

the known colors or dyes impart an objectionable color to the gasoline. Some of the dyes render the gasoline unfit for dry cleaning. Most of the colors or dyes do not impart a fast color to the gasoline, the color changing, say from blue to green, on exposure to light or during storage.

The colors that have been found to most nearly respond to all the requirements are among those which are sometimes classed in the alizarine group and sometimes in the anthraquinone group. There is a vast number of such colors, however, and very few are available that will respond, even in degree, to the requirements hereinbefore mentioned.

Among the colors meeting the above requirements which heretofore have never been successfully imparted to gasoline is a blue color. This color is, on the whole, the most desirable, not only because no inferior gasoline has this color, but also because the color is not suggestive of inferiority in the mind of the public.

Many efforts have been made, without success, to secure a gasoline of this color that will have no objectionable characteristics. In most instances, where gasoline has been satisfactorily colored blue in the first instance, it turns to a green, or greenish blue, or yellow, upon exposure to sunlight or after storage.

After experimenting with and thoroughly testing a great number of colors, I have discovered certain colors that impart to the gasoline the desired blue color and that, in maximum degree, meet all the requirements above enumerated. These colors are derivatives of indigo, specifically certain brominated derivatives or mixtures of brominated derivatives of indigo, and more particularly a mixture of 4.5.7.4'.5'.7' hexabrom indigo, together with 4.5.7.5'.7' pentabrom indigo, commercially known as durindone blue 6 B;

the hexabromindigo having the structural formula—



10 and the pentabromindigo having the structural formula—



15 the hexabrom compound usually being present in a greater proportion than the penta- brom compound, and the mixture usually containing a small proportion of tetrabromindigo (5.7.5'.7').

This color has also the advantage that it 25 has the maximum coloring effect sought when used in the proportion of about one part in about 200,000 parts of gasoline. Gasoline so colored is a beautiful blue free from any cloudy effect. It is so reliably fast 30 that it does not change color when exposed to sunlight for a prolonged period.

The specific color compound desired is a dark blue powder, readily soluble in xylene, benzene, carbon tetrachloride, chloroform, 35 and amyl acetate. It is less soluble in gasoline and almost insoluble in ethyl and in methyl alcohol.

It is insoluble in water.

Its spectrum in xylene ranges in accordance 40 with the percentage of the various components present.

Its insolubility in water is an important characteristic. Most dyes, when mixed with oil, will, when water is subsequently added, 45 leave the oil, in whole or in part, and go into the water. A color that cannot be washed out with water has the additional advantage that it insures against the addition of water to the gasoline, because, if 50 water be added thereto, the buyer can see the water, as a transparent mass against a blue background, flowing through the glass on the pump.

The proportion of the various brominated derivatives of indigo present in the described 55 portion of the pentabrom indigo determines the intensity and the shade of the blue color of the solution.

The pure hexabrom derivative of indigo yields a pure deep blue color. As the proportion 60 of the pentabrom indigo is increased, the color of the solution shades from blue to violet. If more than a trace of tetrabrom indigo is present in the solution, the violet color is intensified.

It will be understood that other haloge-

nated derivatives of indigo having similar properties in regard to color fastness to light and solubility may be employed.

As examples, 5.7.5'.7' dichlorodibrom indigo; 5.7.5'.7' tetrachlorindigo; 4.5.4'.5' dichlorodibrom indigo may be employed with good results, but are less preferable.

It should be understood, however, that the gasoline, when colored with the colors herein described, may not retain the desired color unless, as hereinbefore stated, the gasoline is carefully refined and is substantially water-white in color. Refined gasoline having a yellow tinge will produce a green product. Even if the refined gasoline has no yellow tinge, still, if it is not properly refined, it will become yellow on standing and will eventually turn green. There is, in fact, probably only a minor percentage of gasoline commonly manufactured that 85 will lend itself to being blended with the above color for the purpose of producing blue gasoline.

An example of a process that has been 90 successfully employed for manufacturing water-white gasoline to which a blue color may be permanently imparted by means of the above mentioned dye is the process set forth in the Thomas Patent No. 1,624,692, dated April 12, 1927, for Process of manufacturing gasoline.

It is preferred to add the color to the gasoline by dissolving it in a small quantity of benzol and gradually adding the concentrated solution to the quantity of gasoline 100 intended to be colored. This procedure follows known methods of adding colors or dyes to petroleum products.

Having now fully described my invention, what I claim and desire to protect by Letters Patent is:

1. A colored gasoline comprising commercial gasoline containing a small proportion of a halogenated derivative of indigo.
2. A colored gasoline comprising commercial gasoline containing a small proportion of a brominated derivative of indigo.
3. A colored gasoline comprising commercial gasoline containing a small proportion of a mixture of halogenated derivatives of indigo.
4. A colored gasoline comprising commercial gasoline containing a small proportion of a mixture of brominated derivatives of indigo.
5. A colored gasoline comprising commercial gasoline containing a small proportion of hexabromindigo.
6. A colored gasoline comprising commercial gasoline containing a small proportion of a mixture of hexabromindigo (4.5.7.4'.5'.7') and of pentabromindigo (4.5.7.5'.7').
7. A colored gasoline comprising commercial gasoline containing a small proportion

of a mixture of hexabromindigo (4.5.7.4'.-5'.7') and of pentabromindigo (4.5.7.5'.7') together with a smaller proportion of tetrabromindigo (5.7.5'.7').

5 In testimony of which invention, I have hereunto set my hand, at Swarthmore, Pennsylvania, on this 26th day of July, 1928.

GELLERT ALLEMAN.

10

15

20

25

30

35

40

45

50

55

60

65